# EUROPEAN PATENT SPECIFICATION

(11) **EP 0 002 923 B1**
(45) Date of publication and mention of the grant of the patent: **11.11.1981**
(21) Application number: 78300851.9
(22) Date of filing: 18.12.1978
(51) Int. Cl.: C22C 19/00, C22C 27/04, C22C 38/00

(54) **Iron group transition metal-refractory metal-boron glassy alloys**
Glasartige Legierungen aus einem oder mehreren Übergangsmetallen der Eisengruppe, einem oder mehreren hochwarmfesten Metallen und Bor
Alliages vitreux comprenant un métal ou des métaux de transition du groupe du fer, un métal ou des métaux réfractaires et du bore

(30) Priority: 03.01.1978 US 866670; 03.01.1978 US 866671; 03.01.1978 US 866675; 27.02.1978 US 881213
(43) Date of publication of application: 11.07.1979
(73) Proprietor: ALLIED CORPORATION, Morristown New Jersey 07960 (US)
(72) Inventor: Ray, Ranjan, Randolph New Jersey 07801 (US)
(74) Representative: Baillie, Iain Cameron

## Description

### BACKGROUND OF THE INVENTION

### 1. Field of the Invention

The invention relates to glassy alloys containing low boron content and molybdenum and/or tungsten in conjunction with at least one other metal of the group cobalt, iron and nickel.

### 2. Description of the Prior Art

Chen et al. in U.S.P. 3,856,513, issued December 24, 1974, have disclosed glassy alloys consisting essentially of about 60 to 90 atom percent of at least one element of iron, nickel, cobalt, vanadium and chromium, about 10 to 30 atom percent of at least one element of phosphorus, boron and carbon and about 0.1 to 15 atom percent of at least one element of aluminum, silicon, tin, germanium, indium, antimony and beryllium. Up to about one-fourth of the metal may be replaced by elements which commonly alloy with iron and nickel, such as molybdenum, titanium, manganese, tungsten, zirconium, hafnium and copper. Chen et al. also disclose wires of glassy alloys having the general formula T_{;}X_{;}, where T is a transition metal and X is an element selected from the group consisting of phosphorus, boron, carbon, aluminum, silicon, tin, germanium, indium, beryllium and antimony, and where "i" ranges from about 70 to 87 atom percent and "j" ranges from about 13 to 30 atom percent.

More recently, Masumoto et al. in U.S.P. 3,986,867 issued October 19, 1976, have disclosed iron-chromium glassy alloys consisting essentially of about 1 to 40 atom percent chromium, 7 to 35 atom percent of at least one of carbon, boron and phosphorus and the balance iron. Up to about 40 atom percent of at least one of nickel and cobalt, up to 20 atom percent of at least one of molybdenum, zirconium, titanium and manganese and up to about 10 atom percent of at least one of vanadium, niobium, tungsten, tantalum and copper may also be employed. Elements useful for improving mechanical properties include molybdenum, zirconium, titanium, vanadium, niobium, tantalum, tungsten, copper and manganese, while elements effective for improving the heat resistance include molybdenum, zirconium, titanium, vanadium, niobium, tantalum and tungsten.

French specification 2,281,434 relates to amorphus i.e. glassy alloys containing mixtures of metalloids and metals including alloys containing both phosphorus and boron. French specification 2,317,370 also discloses alloys containing molybdenum or tungsten and at least 15% of metalloid in a glassy alloy.

Efforts to develop new compositions which are easily formed in the glassy state with superior mechanical properties and which at the same time retain high thermal stability are continuing. Substantial amounts of metalloid elements (typically 15 to 25 atom percent) are usually found most suitable for producing the glassy state under reasonable quenching conditions of at least about 10^{so}/sec, consistent with forming a ductile product. However, such high metalloid content combined with a high refractory metal content also may result in increasing brittleness of the glassy alloy in the as-quenched state.

### SUMMARY OF THE INVENTION

In accordance with the invention, substantially totally glassy alloys containing a low boron content as a first component, plus molybdenum or tungsten as a second component in conjunction with one of the metals cobalt, iron and nickel are provided. The glassy alloys of the invention consist essentially of about 5 to 12 atom percent boron, one only of the members selected from the group of 20 to 6Q percent molybdenum and 13 to 40 atom percent tungsten and the balance essentially one of the group iron, cobalt and nickel. In a more specific embodiment glassy alloys containing all three of the metals cobalt, iron and nickel with the above specified boron and second component molybdenum, tungsten and mixtures thereof are provided wherein each of the metals cobalt, iron and nickel is present in an amount of at least about 5 atom percent, plus incidental impurities. The alloys of the invention evidence hardness values of at least about 1000 Kg/mm³, ultimate tensile strengths of at least about 2275 MPa (330 Kpsi) and crystallization temperatures of at least about 445°C.

### DETAILED DESCRIPTION OF THE INVENTION

The glassy alloys of the invention consist essentially of (I) about 5 to 12 atom percent boron together with (II) one only of the group consisting of molybdenum (about 20 to 60 wt%) and tungsten (about 13 to 40 wt%) with the balance being one of the group iron, cobalt and nickel or (III) glassy alloys containing at least 5 atom percent of all three metals, cobalt, iron and nickel in amounts of at least 5 atom percent wherein the amount of molybdenum, tungsten or mixtures thereof, is used in lesser quantities of about 5 to 15 atom percent together with boron in specified amounts of 5 to 12 atom percent. Preferably the boron is present in amounts of 8 to 10 atom percent and the molybdenum and tungsten as component II in amounts of 30 to 50 atom percent and as component III in amounts of 8 to 12 atom percent. Examples of glassy alloys of the invention include

It is seen that the glassy metal alloys of the invention comprise three components: the first component is boron in amounts of from about 5 to about 12 atom percent; the second component is a refractory metal of the group molybdenum in amounts of 20 to 60 atom percent and tungsten in amounts of from about 13 to 40 atom percent; and the third component comprising the balance of the alloy is selected from the group cobalt, iron and nickel.

The low boron content, the refractory metal content and the third component are interdependent. When the boron content is less than about 5 atom percent and both the refractory metal content and the iron group metal content lie within the limits specified, rapidly quenched ribbons are not totally glassy. Rather, the rapidly quenched ribbons contain crystalline phases, which may comprise a substantial fraction of the material, depending on specific composition. The rapidly quenched ribbons containing crystalline phases or mixtures of both glassy and crystalline phases have inferior mechanical properties, i.e., low tensile strength, and are brittle. Typically, such ribbons, having thicknesses up to 38 11m (0.0015 inch), will fracture if bent to a radius of curvature less than 100 times the thickness.

When the boron content is greater than about 13 atom percent and both the refractory metal content and the iron group metal content lie within the limits specified, rapidly quenched ribbons, while remaining fully glassy are, nevertheless, more brittle than ribbons having compositions within the scope invention. Typically, such ribbons fracture when bent to a radius of curvature less than about 100 times the thickness.

Similarly, for refractory metal concentrations less than those listed above, compositions containing such low metalloid content do not form glassy alloys at the usual quench rates. For refractory metal concentrations greater than those listed above, compositions containing such low metalloid content form brittle glassy alloys. If the alloys do not contain these metals in the respective proportions then, in general, the alloys do not form fully glassy ductile ribbons.

In contrast, when the boron content ranges from about 5 to 12 together with the specified proportions of the refractory metal, molybdenum and/or tungsten, second component together with the third component of the_{'} group iron, cobalt and nickel, rapidly quenched ribbons are substantially totally glassy and possess superior mechanical properties, i.e., high tensile strength and ductility. For example, glassy ribbons of the invention can be bent without fracture to a radius of curvature about 10 times the thickness.

Use of refractory metal elements other than molybdenum and tungsten and use of metalloids other than boron in the amounts given do not form ductile glassy alloys at the usual quench rates. For example, replacing boron by carbon or silicon results in the formation of crystalline, rather than glassy, phases.

The purity of all elements is that found in normal commercial practice. However, it is contemplated that minor additions (up to a few atom percent) of other alloying elements may be made without an unacceptable reduction of the desired properties. Such additions may be made, for example, to aid the glass-forming behavior. Such alloying elements include the transition metal elements (Groups IB to VIIB and VIII, Rows 4, 5 and 6 of the Periodic Table, other than the elements mentioned above) and metalloid elements (carbon, silicon, aluminum, and phosphorus), the amounts, as already made clear must not be such as to interfere with the essential components of the alloy.

The thermal stability of a glassy alloy is an important property in certain applications. Thermal stability is characterized by the time-temperature behavior of an alloy, and may be determined in part by differential thermal analysis (DTA). Glassy alloys with similar crystallization behavior as observed by DTA may exhibit different embrittlement behavior upon exposure to the same heat treatment cycle. By DTA measurement, crystallization temperatures Tₑ can be accurately determined by heating a glassy alloy (at about 20° to 50°C/min) and noting whether excess heat is evolved over a limited temperature range (crystallization temperature) or whether excess heat is absorbed over a particular temperature range (glass transition temperature). In general, the glass transition temperature is near the lowest, or first, crystallization temperature Tₑₗ and, as is conventional, is the temperature at which the viscosity ranges from about 10¹² to 10¹³ Pas (10¹³ to 10¹⁴ poise).

The glassy alloys of the invention are formed by quenching an alloy melt of the appropriate composition at a rate of at least about 10⁵°C/sec. A variety of techniques are available, as is well-known in the art, for fabricating rapidly-quenched continuous filament. Typically, a particular composition is selected, powders of the requisite elements (or of materials that decompose to form the elements) in the desired proportions are melted and homogenized, and the molten alloy is rapidly quenched on a chill surface, such as a rapidly rotating cylinder.

The alloys of the invention are substantially totally glassy, as determined by X-ray diffraction. The term "glassy", as used herein, means a state of matter in which the component atoms are arranged in a disorderly array; that is, there is no long range order. Such a glassy alloy material gives rise to broad, diffuse diffraction peaks when subjected to electromagnetic radiation in the X-ray region (about 0.01 to 50 A wavelength). This is in contrast to crystalline material, in which the component atoms are arranged in an orderly array, giving rise to sharp diffractions peaks. The term "substantially totally glassy" as used herein means a state of matter having crystalline and amorphous phases, the amorphous phase constituting at least about 80 percent of the combined phases. Thermal stability of the alloys improves as the degree of amorphousness thereof approaches 100%. Accordingly, totally glassy alloys, possessing a single, amorphous phase constituting 100% of the component atoms are preferred.

The glassy alloys of the invention evidence hardness values of at least about 1000 kg/mm², ultimate tensile strengths of at least about 2413 MPa(350 Kpsi) and crystallization temperatures of at least about 445°C. Preferred alloy compositions consist essentially of about 50 to 65 atom percent of one of the iron group metals of iron, cobalt and nickel, about 13 to 35 atom percent of the remaining two iron group metals, about 8 to 12 atom percent of at least one of molybdenum and tungsten and about 8 to 10 atom percent boron. The alloys having such preferred compositions are especially capable of being fabricated as good quality, ductile ribbons exhibiting high tensile strength.

The high mechanical strength and high thermal stability of the glassy alloys of the invention render them suitable for use as reinforcement in composites for high temperature applications.

### Examples

Alloys were prepared from constituent elements of high purity (99.9%). The elements with a total weight of 30 g were melted by induction heater in a quartz crucible under vacuum of 133 mPa (10-³ Torr). The molten alloy was held at 150° to 200°C above the liquidus temperature for 10 min and allowed to become completely homogenized before it was slowly cooled to the solid state at room temperature. The alloy was fractured and examined for complete homogenity.

About 10 g of the alloys was remelted to 150°C above liquidus temperatures under vacuum of 133 mPa (10-³ Torr) in a quartz crucible having an orifice of 254 ,um (0.010 inch) diameter in the bottom. The chill substrate used in the present work was beryllium-copper alloy in a heat-treated condition having moderately high strength and thermal conductivity. The substrate material contained 0.4 to 0.7 wt% beryllium, 2.4 to 2.7 wt% cobalt and copper as balance. The substrate was kept rotating at a surface speed of 20.3 m/s (4000 ft/min). The substrate and the crucible were contained inside a vacuum chamber evacuated to 133 mPa (10-³ Torr).

The melt was spun as a molten jet by applying argon pressure of 34.5 kPa (5 psi) over the melt. The molten jet impinged vertically onto the internal surface of the rotating substrate. The chill-cast ribbon was maintained in good contact with the substrate by the centrifugal force acting on the ribbon against the surface. The ribbon was ejected off the substrate by nitrogen gas at 207 kPa (30 psi), two- thirds circumferential length away from the point of jet impingement. During the metallic glass ribbon casting operation, the vacuum chamber was maintained under a dynamic vacuum of 2.7 kPa (20 Torr). The substrate surface was polished with 320 grit emery paper and cleaned and dried with acetone prior to the start of the casting operation. The as-cast ribbons were found to have good edges and surfaces. The ribbons had the following dimensions: 25.4 to 30.5,um (0.0001 to 0.0012 inch) thickness and 381 pm to 508!1m (0.015 to 0.020 inch) width.

The degree of glassiness was determined by X-ray diffraction. A cooling rate of at least about 10⁵°C/sec was attained by the quenching process.

Hardness was measured by the diamond pyramid tehcnique using a Vickers-type indenter, consisting of a diamond in the form of a square-base pyramid with an included angle of 136° between opposite faces. Loads of 100 g were applied. Crystallization temperature was measured by differential thermal analysis at a scan rate of about 20°C/min. Ultimate tensile strength was measured on an Instron machine using ribbons with unpolished edges. The gauge length of the specimens was 25.4 mm (1 inch) and the cross-head speed was 8.46,ums/s (0.02 in/min).

The following values of hardness in kg/mm², ultimate tensile strength in MPa (Kpsi) and crystallization temperature in °C, listed in Tables I-IV below, were measured for a number of compositions falling within the scope of the invention.

Table V sets forth compositions outside the scope of the invention and the results of structural analysis by X-ray diffraction in chill cast ribbons of these compositions prepared as above, and the brittleness of the ribbons.

## Claims

1. A substantially totally glassy alloy as herein defined containing molybdenum or tungsten and a metalloid characterised in that the alloy consists essentially of (I) 5 to 12 atom percent boron and either (II) at least one of 20 to 60 atom percent molybdenum and 13 to 40 atom percent tungsten, with the balance being essentially at least one of cobalt, iron and nickel; or (III) at least one of 5 to 15 atom percent molybdenum, tungsten or a mixture thereof and the balance being essentially iron, cobalt and nickel with each being present in an amount of at least 5 atom percent.

2. The glassy alloy of claim 1 wherein the boron is present in an amount of 8-10 atom percent, the molybdenum and tungsten in Member II is present in amounts of 30 to 50 atom percent and 30 to 40 atom percent respectively and the molybdenum and tungsten in Member III is present in amounts of 8 to 12 atom percent.

3. A substantially totally glassy alloy according to claim 1 consisting essentially of 5 to 12 atom percent boron, at least one of 30 to 60 atom percent molybdenum and 20 to 35 atom percent tungsten and the balance essentially nickel.

4. The glassy alloy of claim 3 having a composition selected from the group consisting of Ni₅₇Mo₃₅B₈, Ni₅₅Mo₃₅B₁₀, Ni₅₀Mo₄₀B₁₀, Ni₄₅Mo₄₅B₁₀, Ni₄₂Mo₅₀B₈,Ni₇₀W₂₂B₈, Ni₇₀W₂₀B₁₀ and Ni₆₀W₃₀B₁₀.

5. A substantially totally glassy alloy according to claim 1 consisting essentially of 5 to 12 atom percent boron, at least one of 25 to 40 atom percent molybdenum and 13 to 25 atom percent tungsten and the balance essentially iron.

6. The glassy alloy of claim 5 having a composition selected from the group consisting of Fe₆₀Mo₃₀B₁₀, Fe₅₅Mo₃₅B₁₀, Fe₇₇W₁₅B₈ and Fe₇₇W₁₃B₁₀.

7. A substantially totally glassy alloy according to claim 1 consisting essentially of 5 to 12 atom percent boron, at least one of 20 to 50 atom percent molybdenum and 15 to 40 atom percent tungsten and the balance essentially cobalt.

8. The glassy alloy of claim 7 having a composition selected from the group consisting of Co₆₆Mo₂₆B₈, Co₅₅Mo₃₅B₁₀, Co₅₀Mo₄₀B₁₀, Co₇₀W₂₀B₁₀ and Co₆₀W₃₀B₁₀.

9. A substantially totally glassy alloy according to claim 1 consisting essentially of 5 to 10 atom percent boron, 5 to 15 atom percent of at least one of molybdenum and tungsten and the balance essentially iron, cobalt and nickel, each present in an amount of at least 5 atom percent.

10. The glassy alloy of claims 9 consisting essentially of 8 to 10 atom percent boron, 8 to 12 atom percent of at least one of molybdenum and tungsten, 50 to 65 atom percent of one of the iron group metals and 13 to 35 atom percent of the remaining two of the iron group metals.

## Revendications

1. Alliage vitreux de façon sensiblement totale, tel que défini dans la description, contenant du molybdène ou du tungstène et un métalloïde caractérisé en ce que l'alliage est constitué essentiellement de (1) 5 à 12% atomes de bore et soit (II) au moins l'un des métaux choisis parmi le molybdène à raison de 20 à 60% en atomes et le tungstène à raison de 13 à 40% en atomes, le restant étant essentiellement au moins l'un des métaux choisis parmi le cobalt, le fer et le nickel, soit (III) au moins l'un des métaux choisis parmi le molybdène et le tungstène à raison de 5 à 15% en atomes ou un mélange de ces derniers métaux et le restant étant essentiellement du fer, du cobalt et du nickel dont chacun est présent en une quantité d'au moins 5% en atomes.

2. Alliage vitreux selon la revendication 1, dans lequel le bore est présent en une quantité de 8-10% en atomes, le molybdène et le tungstène du groupe II est présent respectivement en quantités de 30 à 50% en atomes et 30 à 40% en atomes et le molybdène et le tungstène du groupe III est présent en quantités de 8 à 12% en atomes.

3. Alliage vitreux de façon sensiblement totale selon la revendication 1, comprenant essentiellement 5 à 12% en atomes de bore, au moins l'un métaux le molybdène à raison de 30 à 65% en atomes et le tungstène à raison de 20 à 35% en atomes, le restant étant essentiellement du nickel.

4. Alliage vitreux selon la revendication 3 ayant une composition choisie dans le groupe comprenant Ni₅₇Mo₃₅B₈, Ni₅₅Mo₃₅B₁₀, Ni₅₀Mo₄₀B₁₀, Ni₄₅Mo₄₅B₁₀, Ni₄₂Mo₅₀B₈, Ni₇₀W₂₂B₈, Ni₇₀W₂₀B₁₀ et Ni₆₀W₃₀B₁₀.

5. Alliage vitreux de façon sensiblement totale selon la revendication 1, comprenant essentiellement de 5 à 12% en atomes de bore, au moins l'un des métaux le molybdène à raison de 25 à 45% en atomes et le tungstène à raison de 12 à 25% en atomes, le restant étant essentiellement du fer.

6. Alliage vitreux selon la revendication 5, ayant une composition choisie parmie les groupes comprenant Fe₆₀Mo₃₀B₁₀, Fe₅₅Mo₃₅B₁₀, Fe₇₇W₁₅B₈, Fe₇₇W₁₃B₁₀·

7. Alliage vitreux de façon sensiblement totale selon la revendication 1, comprenant essentiellement de 5 à 12% en atomes de bore, au moins l'un des métaux choisis parmi le molybdène à raison de 20 à 50% en atomes et le tungstène à raison de 15 5 à 45% en atomes, le restant étant essentiellement du cobalt.

8. Alliage vitreux selon la revendication 7, ayant une composition choisie parmi le groupe comprenant Co₆₆Mo₂₆B₈, Co₅₅Mo₃₅B₁₀, Co₅₀Mo₄₀B₁₀, Co₇₀W₂₀B₁₀, Co₆₀W₃₀B₁₀.

9. Alliage vitreux de façon sensiblement totale selon la revendication 1, comprenant essentiellement de 5 à 10% en atomes de bore, 5 à 15% en atomes d'au moins l'un des métaux choisis parmi le molybdène et le tungstène et le restant étant essentiellement constitué par du fer, du cobalt et du nickel, chacun présent en une quantité d'au moins 5% en atomes.

10. Alliage vitreus selon la revendication 9 comprenant essentiellement de 8 à 10% en atomes de bore, 8 à 12% en atomes d'au moins l'un des métaux choisis parmi le molybdène et le tungstène, 50 à 65% en atomes de l'un des métaux du groupe du fer et 13 à 35% en atomes des deux métaux restants du groupe des métaux du fer.

## Patentansprüche

1. Im wesentlichen vollständig glasartige Legierung der hier definierten Art, die Molybdän oder Wolfram und ein Nichtmetall enthält, dadurch gekennzeichnet, daß die Legierung im wesentlichen aus (I) 5 bis 12 Atomprozent Bor und entweder (11) mindestens einer der Komponenten 20 bis 60 Atomprozent Molybdän und 13 bis 40 Atomprozent Wolfram, Rest im wesentlichen eins der Elemente Kobalt, Eisen und Nickel; oder (111) mindestens einer der Komponenten 5 bis 15 Atomprozent Molybdän, Wolfram oder ein Gemisch derselben, Rest im wesentlichen Eisen, Kobalt und Nickel in einer Menge von je mindestens 5 Atomprozent; besteht.

2. Glasartige Legierung nach Anspruch 1 dadurch gekennzeichnet, daß das Bor in einer Menge von 8 bis 10 Atomprozent vorhanden ist und daß das Molybdän und das Wolfram in dem Anteil 11 in Mengen von 30 bis 50 Atomprozent bzw 30 bis 40 Atomprozent und das Molybdän und das Wolfram in dem Anteil 111 in Mengen von 8 bis 12 Atomprozent vorhanden sind.

3. Glasartige Legierung nach Anspruch 1, die sie im wesentlichen aus 5 bis 12 Atomprozent Bor, mindestens einer der Komponenten 30 bis 60 Atomprozent Molybdän und 20 bis 35 Atomprozent Wolfram, Rest im wesentlichen Nickel, besteht.

4. Glasartige Legierung nach Anspruch 3, welche die Zusammensetzung Ni₅₇Mo₃₅B₈ oder Ni₅₅Mo₃₅B₁₀ oder Ni₅₀Mo₄₀B₁₀ oder Ni₄₅Mo₄₅B₁₀ oder Ni₄₂MoₛₒBₛ oder Ni₇₀W₂₂B₈ oder Ni₇₀W₂₀B₁₀ oder Ni₆₀W₃₀B₁₀ hat.

5. Im wesentlichen vollständig glasartige Legierung nach Anspruch 1, die im wesentlichen aus 5 bis 12 Atomprozent Bor, mindestens einer der Komponenten 25 bis 40 Atomprozent Molybdän und 13 bis 25 Atomprozent Wolfram, Rest im wesentlichen Eisen, besteht.

6. Glasartige Legierung nach Anspruch 5, welche die Zusammensetzung Fe₆₀Mo₃₀B₁₀ oder Fe₅₅Mo₃₅B₁ₒ oder Fe₇₇W₁₅B₈ oder Fe₇₇W₁₃B₁₀ hat.

7. Im wesentlichen vollständig glasartige Legierung nach Anspruch 1, die im wesentlichen aus 5 bis 12 Atomprozent Bor, mindestens einer der Komponenten 20 bis 50 Atomprozent Molybdän und 15 bis 40 Atomprozent Wolfram, Rest im wesentlichen Kobalt, besteht.

8. Glasartige Legierung nach Anspruch 7, welche die Zusammensetzung Co₆₆Mo₂₆B₈ oder Co₅₅Mo₃₅B₁₀ oder Co₅₀Mo₄₀B₁₀ oder Co₇₀W₂₀B₁₀ oder Co₆₀W₃₀B₁₀ hat.

9. Im wesentlichen vollständig glasartige Legierung nach Anspruch 1, die im wesentlichen aus 5 bis 10 Atomprozent Bor, 5 bis 15 Atomprozent wenigstens einer der Komponenten Molybdän und Wolfram, Rest im wesentlichen Eisen, Kobalt und Nickel in einer Menge von je mindestens 5 Atomprozent besteht.

10. Glasartige Legierung nach Anspruch 9, die im wesentlichen aus 8 bis 10 Atomprozent Bor, 8 bis 12 Atomprozent mindestens einer der Komponenten Molybdän und Wolfram. 50 bis 65 Atomprozent eines Metalls der Eisengruppe und 13 bis 35 Atomprozent der übrigen zwei Metalle der Eisengruppe besteht.
